

## UNITED STATES PATENT OFFICE

2,650,901

## ELECTROPLATING ON ALUMINUM

**Kuno L. van der Horst, Portville, N. Y., assignor  
to Van der Horst Corporation of America,  
Olean, N. Y., a corporation of Delaware**

**No Drawing. Application June 8, 1949,  
Serial No. 97,912**

**7 Claims. (Cl. 204—33)**

**1**

This invention relates to electroplating on aluminum, and more particularly to the preparation of aluminum articles for the electroplating of a metal thereon and especially the electroplating of chromium on the aluminum.

The invention is applicable not only to aluminum itself as the base or foundation metal, such as the product of the Aluminum Corporation of America known as 2S which is sold as commercially pure aluminum and of which some 99% or more is aluminum metal, but also to common commercial aluminum alloys as well, i. e. those alloys which are predominantly aluminum; for example, such aluminum alloys of the Aluminum Corporation of America as the wrought aluminum alloys identified as 24S (having 4.5% copper, 1.5% magnesium, and 0.6% manganese), and 75S (1.6% copper, 2.5% magnesium, 5.6% zinc, and 0.3% chromium); the die casting aluminum alloy identified as 380 (having 3.5% copper and 9.0% silicon); and the sand casting alloys identified as 355 (1.3% copper, 5.0% silicon, and 0.5% magnesium) and 356 (7% silicon and 0.3% magnesium). Accordingly in this specification and its claims the word "aluminum" is used in a generic sense, i. e. as including both pure aluminum and those alloys which are predominantly aluminum, except as the contrary may appear.

Heretofore various methods have been proposed for plating on aluminum. Generally at least, each of these includes a series of steps for preparing the aluminum article for the subsequent electrodeposition of the desired metal. In some instances the preparatory steps include an alkaline-etch cleaning operation at an elevated temperature, around 180° F. or more, the purpose of which is to remove the layer of oxide which occurs naturally on all commercial aluminum. Also where chromium is to be electrodeposited on aluminum, at least one plating method used heretofore includes, as a final preparatory step, the electrodeposition of copper on the aluminum, evidently to serve as a bonding metal between the aluminum base and the chromium plate. All the prior practices, so far as I am aware, have undesirable features, and in particular the obtaining of a bond between aluminum and chromium adequate to permit the use of a chromium plate for wear resistance, is, in repetitive factory practice, somewhat difficult and uncertain, or is expensive.

The present invention provides for plating on aluminum with a strong adhesion or bond between the plate and the aluminum surface under production conditions, e. g. a bond sufficient to permit the electroplating of chromium on alu-

**2**

minum for wear resistance purposes. Also in contrast to at least some prior processes, the invention reduces the number of steps preceding the actual electrodeposition of the desired plating metal; for example, it is not necessary, with the invention, to plate the aluminum with copper before depositing chromium.

The invention secures these results by a certain distinctive operation or operations preparatory to the electrodeposition of the metal on the aluminum base metal. Basically this or these preparatory operations comprise subjecting the aluminum or such area or areas of the aluminum as are to be plated, and preferably after having degreased or otherwise cleansed the area or areas to be plated, to vapor blasting until the adherent film of oxide that is found on commercial aluminum has been thoroughly broken down, and preferably, in addition, a fine roughness imparted to or developed on the aluminum surface, or subjecting the area or areas to be plated to another physical treatment, or as it may be called, mechanical treatment, that yields the same results, and also, and advantageously following such physical treatment, subjecting the area or areas to the action of a solution containing caustic alkali and alkali zincate. These primary or basic treatments alone are sufficient to permit the ready plating with a strong bond on some of the common aluminum alloys, or some of the alloys under certain conditions, and may be followed directly by the electrodeposition of the desired metal in, say, the ordinary way. However by adding to these primary or basic treatments an additional step consisting of subjecting the area or areas to be plated to a solution or solutions of a strong mineral acid or acids, e. g. nitric or both sulphuric and nitric, following the physical treatment and prior to the alkali and zincate treatment, not only is the process adapted for plating on the same alloys as before, and the same alloys under the same conditions, but also the process is adapted for plating on still other alloys. Also by adding a still further treatment, i. e. treatment of the physically treated surfaces with caustic alkali and alkali zincate prior to the treatment with a strong mineral acid or acids, still further alloys are added to the field of the process. This last form of the process (i. e. physical treatment, treatment with caustic alkali and zincate, treatment with mineral acid, and then a second treatment with caustic alkali and zincate) appears to be capable of preparing substantially all the common commercial aluminum alloys for the reception of electroplates, and especially for the reception of electroplates of chromium. It will

be understood that no preparatory or intermediate plating step is required with my present invention, at least usually. That is to say, after such preparatory steps as indicated above the metal desired for the plate is electrodeposited directly on the aluminum article, at least usually. Also usually each treatment, or at least each chemical treatment, is followed by a water rinse to wash away matter that may be adhering to the surface as is customary in plating practice, including, usually, a water rinse after the final treatment with caustic alkali and alkali zincate solution and prior to electrodepositing the metal of the plate that is desired.

The steps or treatments described above may follow one another immediately, or with only such little delay between each two as is consistent with convenient shop practices. On the other hand, after the rinsing which follows the physical treatment the treated article can be set aside many hours, if desired, say up to twenty-four hours, before being subjected to the next step or treatment (which, of course, may be either an alkali-zincate or an acid treatment). Likewise after the rinsing following an alkali-zincate treatment, the next treatment (either an acid treatment or the electroplating) can be delayed many hours. Also a delay may be interposed between the rinsing which follows the completion of the acid treatment and the subsequent alkali-zincate treatment, but in this case the permissible delay is generally shorter; say up to one hour. During such intervals the aluminum can be allowed to stand in the open air. However if the atmosphere contains considerable dust or other foreign matter that tends to deposit on the aluminum, the permissible intervals between steps or treatment are shortened thereby. Any oxide that may form on the treated aluminum surfaces during such intervals between treatments seems to have no detrimental effects.

Now taking up the foregoing matters in greater detail:

As before indicated, usually it is necessary or desirable to clean and degrease the aluminum before undertaking plating operations in order to remove the soil and grease that have accumulated on it from handling and previous manufacturing operations. The manner in which this is done is immaterial, speaking generally, e. g. provided the operations are such as produce no detrimental chemical change in the aluminum surfaces. Degreasing by the commonly used vapor degreasing operations wherein the articles are exposed to the vapors of highly volatile solvents, e. g. vapors of the ethylene polychlorides such as ethylene dichloride, trichlorethylene, perchloroethylene and the like, is satisfactory. Usually at least the aluminum article is rinsed with water after the degreasing and cleaning.

The aluminum articles are then ready for the operations of the invention. As before indicated, the first step of the invention is, or includes, a physical treatment which may be by vapor blasting and preferably is by vapor blasting. That is, the whole or such parts or areas of the articles as are to receive the electroplate are subjected to vapor blasting until the surface film of adherent aluminum oxide on these parts or areas has been thoroughly broken down and an apparently new surface exposed, preferably finely roughened. For example, the roughening may be such that its individual depressions are invisible to the eye, but under a magnification of the order of five hundred diameters or more the surface seems to

consist of small irregularly shaped and irregularly overlapping pits or other indentations. Such a blasting effect can be obtained, for example, by using as the grit the crushed siliceous rock of Arkansas known as Novaculite, the grit being of 100 mesh size (which grit has diameters ranging from about 0.0005 to about 0.03 inch), or 1250 mesh size (grit ranging in diameter from about 0.00015 to about 0.00025 inch), or of an intermediate size, or mixtures of such grits, and being suspended in a liquid, for example water (say from 4 to 5 pounds of the grit to each gallon of the liquid), and the mixture being driven toward the aluminum from an internally-cylindrical nozzle having an orifice about one-quarter inch in diameter delivering the mixture at an angle of about 45° to 90° to the area or parts to be plated at a distance of about one-half inch or more therefrom, the mixture being delivered to the nozzle under a head of about 4 feet, and sufficient air being supplied to the liquid passage leading to the nozzle, at a pressure of about 100 pounds per square inch, for delivery from the nozzle with the liquid-grit mixture, to discharge about three-fourths of a gallon of the liquid-grit mixture from the nozzle per minute, and continuing such blasting until the initial oxide film that is on the area or parts to be plated is completely broken down and an apparently new and finely roughened surface produced or developed. Further, a suitable degree of blasting can be determined by the action of the blasted surface in an alkali-zincate solution such as that here described. I. e. if submerging the blasted surface in the alkali-zincate solution results in no or only a small evolution of gas and a substantially immediate deposit of zinc over the whole surface, the blasting has been sufficient and not excessive; on the other hand if the gas evolution is profuse or the zinc coating laid down on the blasted surface is porous (microscopically), the blasting is improper. Where the surface or area to be treated is large, the article may be moved about transversely of the mixture stream during the blasting so as to subject the various parts of a large area to the stream from the nozzle intermittently, or more than one nozzle, discharging to different parts of the article, may be used simultaneously, or both, and thereby the time required for the necessary degree of vapor blasting shortened accordingly. Obviously the time required to produce a new surface by such means in any instance will depend on the size of the area or areas being treated, the number of nozzles employed, etc. However the foregoing is subject to great variation, and accordingly this example is to be regarded only as illustrative of the type of physical treatment that I prefer and a procedure that produces a surface that is illustrative of the type of surface here concerned. Any physical treatment that produces a surface of the same type can be substituted.

Usually the aluminum is rinsed immediately after the physical treatment, say in water, to remove any remnants of the treatment that may remain on it.

Generally the alkali and zincate solution (and each of them, if more than one alkali and zincate treatment is employed), is an aqueous solution, and conveniently the zincate has the same alkali metal as the caustic alkali. Any of the caustic alkalis can be used, such as caustic soda, caustic potash, and the like. I prefer sodium hydroxide. The concentration of the caustic alkali is sufficient to retain the zincate in solution during stor-

before becoming so contaminated that it is best to discard it and start anew. Treatment with such nitric acid solutions may be at, say, substantially room temperature. When a treatment with such an acid solution follows a treatment of an aluminum article with an alkali and zincate treatment, the acid solution treatment is continued until the layer of zinc deposited from the zincate has disappeared. In those instances where the acid treatment follows immediately after the vapor blasting or other physical treatment, the acid solution treatment is continued for anywhere from about ten (10) seconds to one (1) hour or even longer. Speaking generally, a relatively short treatment is required with low concentrations and longer treatments with higher concentrations. The acid treatment may be by spraying, hosing, etc., but I prefer immersion. With a nitric acid concentration of about twenty-five (25) parts to seventy-five (75) parts of water, and at room temperature, immersion for about fifteen (15) seconds is satisfactory when vapor blasting next precedes the acid treatment, and for about thirty (30) seconds is satisfactory when an alkali and zincate treatment next precedes the acid treatment.

As an example of the procedure when an acid treatment is added to the primary physical alkali-zincate treatments: Take an article made of the alloy 380, or one made of alloy 356 or the substantially pure aluminum 2S. Clean this article, rinse in water, and then vapor blast it, and again rinse in water, all as described in the former example of plating on the 380 alloy. Then immerse the article in a solution of 42° Bé. nitric acid twenty-five (25) parts and water seventy-five (75) parts, by volume, at room temperature, for fifteen (15) seconds or a little longer. Then rinse with water. Then immerse in a solution of thirty-five (35) parts of sodium hydroxide, seven (7) parts of sodium zincate and fifty-eight (58) parts of water, by weight, for two (2) minutes at room temperature, and then again rinse in water. The article is then ready for plating. It can be plated with, say, chromium, e. g. by the plating procedure of the former example.

Again, where the acid solution is a mixed acid solution of nitric acid ( $HNO_3$ ) and sulphuric acid ( $H_2SO_4$ ) in water, the quantity of nitric acid to the total quantity of the solution, by volume, may be within substantially the same range as where nitric acid alone is used in the solution. That is, the proportions may be, by volume, between about five (5) and about seventy (70) parts of nitric acid to each one hundred (100) parts of the solution; preferably between about fifteen (15) parts and about sixty-five (65) parts of nitric acid to each one hundred (100) parts of the solution. By volume, between about twelve per cent (12%) and ninety per cent (90%) of the balance of the solution may consist of 66° Bé. sulphuric acid, the remainder being water. Thus for example, a solution consisting of about sixty-one (61) parts of 66° Bé. sulphuric acid, thirty-one (31) parts of 42° Bé. nitric acid, and eight (8) parts of water, by volume, gives substantially uniformly satisfactory results with various alloys. Also a solution consisting of ten (10) parts of 66° Bé. sulphuric acid, twenty-five (25) parts of 42° Bé. nitric acid, and sixty-five (65) parts of water, all by volume, is substantially uniformly satisfactory for many alloys, at least when a treatment with the alkali and zincate solution is interposed between the vapor blasting or other physical treatment and the acid treatment.

Treatment by such a mixed acid solution can be, as with single acid solutions, by hosing, spraying, or otherwise, and preferably is by immersion, and may be at room temperature. When the mixed acid treatment follows immediately after the physical treatment (and water rinsing), subjection of the aluminum to the mixed acid solution for fifteen (15) seconds usually is sufficient, but the time is not critical; when it is preceded by an alkali and zincate treatment, the mixed acid treatment is carried on until the zincate coating on the article disappears.

As an alternative to treatment with a mixed acid solution as just described, the aluminum may be treated with the multiple acids successively, and preferably first with a sulphuric acid solution and then with a nitric acid solution. The nitric acid solution in such cases may be the same as the nitric acid solution described above. The sulphuric acid solution may be between something less than ten (10) parts of 66° Bé. sulphuric acid to ninety (90) parts of water or a little more, and something more than fifty (50) parts of the 66° Bé. acid to fifty (50) parts of water or less, all by volume. When the sulphuric acid concentration is sufficiently high, black streaks tend to form on the aluminum, at least at the higher temperatures, and this should be avoided. As with the other acid solutions, the treatment with a sulphuric acid solution may be by hosing, spraying, etc., but preferably is by immersion. Treatment for a fraction of a minute by each acid, at room temperature, usually is sufficient.

Speaking generally, a good bond can be obtained between, say, electrodeposited chromium and various of the aluminum alloys when an acid solution containing nitric as the sole acid is used, especially if the acid treatment is preceded (as well as followed) by an alkali and zincate treatment, but the action of such an acid solution is not so satisfactory with some alloys as with others. For example, where the alloy contains both magnesium and silicon, usually at least it is either necessary or desirable to treat the article with both sulphuric acid and nitric acid. To this end the article can be treated first with a solution of sulphuric acid and then with a solution of nitric acid, as indicated above, or in the alternative the article can be treated with a solution containing both sulphuric and nitric acids as also described above.

As an example of treatment with two acids, and also an example of two treatments with an alkali-zincate solution: Take an article made of the substantially pure aluminum 2S, or made of one of the alloys 380, 356, 24S, 75S, 355. Clean this article, then rinse it with water, vapor blast it, and again rinse with water, all as described in the first example of plating on 380 alloy above. Then immerse the article in a solution of sodium hydroxide and sodium zincate in water, such as that described in the earlier example, at room temperature, for two minutes or until a film of zinc has been deposited on the article, and again rinse the article with water. Then immerse the article in a solution composed of ten (10) parts of 66° Bé. sulphuric acid, twenty-five (25) parts of 42° Bé. nitric acid, and sixty-five (65) parts of water, by volume, at room temperature, for say thirty (30) seconds or until any zinc coating on the article has disappeared; or as an alternative to such acid treatment, immerse the article in a solution composed of, say, thirty (30) parts of 66° Bé. sulphuric acid and seventy (70) parts

age, and usually to this end is a number of times that of the zincate. The concentrations of the two are such that the solution acts to remove substantially whatever remnants, if any, of aluminum oxide film that otherwise might remain on the surface of the article after the physical treatment or any treatment, whatever it may be, that precedes the alkali-zincate treatment, and also if the interval between an alkali-zincate treatment and whatever treatment may precede the alkali-zincate treatment is sufficiently long to permit the formation of oxide on the aluminum anew, to remove this fresh oxide, and additionally deposit an extremely thin, relatively uniform layer of zinc on the surface, by displacement from the zincate. The interval, if any, between the completion of the preceding treatment and beginning of the alkali-zincate treatment should not be longer, at most, than sufficient to permit the formation of a thin film of oxide of substantially uniform thickness on the aluminum. Speaking generally, the solution may contain from about thirty (30) parts to saturation of the caustic alkali, from about six (6) parts to saturation of the zincate, and sufficient water to make up 100 parts, all by weight. A good solution is one having thirty-five (35) parts of caustic soda ( $NaOH$ ), seven (7) parts of sodium zincate ( $Na_2ZnO_2$ ), and fifty-eight (58) parts of water, all by weight. The treatment of the aluminum articles may be hosing, spraying or otherwise; usually I prefer immersion of the article in the solution as a separate step after rinsing of the article following the preceding step whatever the latter may be. The treatment is continued until substantially the whole of the blasted surface has been covered with a coating of zinc, which may be very thin. With the 35-7-58 solution, immersion for about two minutes at room temperature is sufficient, at least usually. However the immersion time is not critical and can be varied, as will be understood from the foregoing. Sometimes it may be even as little as about one-half minute, and in some circumstances even as short as ten seconds, and it may be for materially longer than two minutes. Generally operation at room temperature appears to be satisfactory, especially with immersion as long as two minutes.

With some aluminum alloys, as indicated above, satisfactory adhesion or bond between the chromium and the base metal is obtained by the physical treatment and a single treatment with such an alkali and zincate solution. An example of this type occurs with the die casting alloy identified above as 380. First cleaning thoroughly, then rinsing with water, and then vapor blasting this aluminum alloy with 1250 mesh Novaculite grit as described above, then immediately water rinsing the article, and immediately thereafter or later immersing for two minutes at room temperature in a solution consisting of thirty-five (35) parts of sodium hydroxide, seven (7) parts of sodium zincate, and fifty-eight (58) parts of water, all by weight, then water rinsing again, and then chromium plating according to ordinary chromium plating practices, gives a good plate and a good bond between the chromium and the alloy. The chromium may be plated, for example, from an aqueous solution made up primarily of about thirty-four (34) ounces of chromic acid ( $CrO_3$ ) and thirty-four one-hundredths (0.34) of an ounce of the sulphate radical ( $SO_4$ ) per gallon and with about one (1) ounce of the chromium in trivalent form, at a temperature of about  $130^{\circ} F.$  and with a current

density of from about one (1) to about six (6) amperes per square inch, using a customary lead anode.

As another example, when any one of aluminum alloys has been plated with chromium and thereafter the plate stripped from the alloy by electrochemical action (i. e. with the plated article as an anode in an electrolyte consisting of a solution of, say, from fifteen (15) to twenty (20) parts of  $66^{\circ} Bé$  sulphuric acid and from eighty-five (85) to eighty (80) parts of water, by weight), the alloy can be replated with chromium with a good strong bond by the same two-step preparatory procedure. With this two-step preparatory operation however, it seems to be more difficult to obtain a good bond when the blasting is done with 100 mesh Novaculite grit than when done with 1250 mesh Novaculite grit. Accordingly with the two-step preparatory procedure I prefer to use a grit finer than 100 mesh and usually I use the 1250 mesh Novaculite or thereabout.

The concentration of acid in the mineral acid solutions is variable over a wide range. For example where the acid is nitric ( $HNO_3$ ), the acid solution may be between about five (5) parts of the  $42^{\circ} Bé$  nitric acid to ninety-five (95) parts of water and about seventy (70) parts of the  $42^{\circ} Bé$  acid to thirty (30) parts of water, all by volume. The nitric acid mentioned throughout this specification is  $42^{\circ} Bé$  acid. However when the lower concentrations, i. e. five (5) parts and somewhat higher, are used on copper-containing alloys, the solution tends to become contaminated with copper rather rapidly so that in even such short periods of continuous use as three or four days, the copper concentration may become so high that on occasion copper will deposit out of the acid solution by displacement onto an article being treated. Such a deposit tends to cause a poor bond between a subsequently applied chromium plate and the aluminum surface. Further, if the acid solution is too dilute, it tends to pit-etch the aluminum if the aluminum is subjected to the solution too long, and during the subsequent treatment of the article with an alkali and zincate solution the zinc tends to build up to too thick a coating, and this also tends to a poor bond. Likewise at the other end of the range, too high a concentration of nitric acid tends to poor results at times at least. For example, when an acid treatment is preceded by an alkali and zincate treatment, an acid concentration of about sixty-five (65) or seventy (70) parts tends to cause the formation of blackish streaks on at least some of the alloys, and the bond between a chromium plate and the aluminum, at the areas occupied by these streaks, tends to be poor. Generally therefore, both to obtain uniformly good results and to avoid having to discard and replace a nitric acid bath too frequently I use in nitric acid baths a nitric acid concentration appreciably higher than ten (10) parts and less than seventy (70) parts, advantageously somewhere between fifteen (15) parts and sixty-five (65) parts, and preferably somewhere around twenty-five (25) parts, the remainder to make up a total of one hundred (100) parts in each instance being water, all by volume. Usually an aqueous solution of about twenty-five (25) parts of nitric acid to seventy-five (75) parts of water, with occasional replenishments of acid and water (usually mostly acid, because drag-in of water from the previous rinsings tends to maintain sufficient water in the solution), can be used for quite a period (say up to five or six weeks of forty working hours each)

of water, by volume, at room temperature, for about one (1) minute, then rinse it with water, and then immerse it in a solution composed of twenty-five (25) parts of 42° Bé. nitric acid and seventy-five (75) parts of water, by volume, at room temperature, for about thirty (30) seconds or at least until any zinc there may have been on the article has disappeared. On the completion of either of these acid treatments, again rinse the article with water, then immerse the article in a solution of sodium hydroxide and sodium zincate in water such as that described in the first example above of plating on alloy 380, at room temperature, for two minutes or until a new film of zinc has been deposited on the article, and then again rinse with water. The article is then ready for plating, and can be plated with chromium, e. g. by the plating procedure of the former example.

It will be understood of course that the invention is not limited to the specific details appearing above except as appears hereafter in the claims.

What I claim is:

1. The method of preparing an aluminum article for electroplating which comprises vapor blasting that portion of the article that is to be plated, with a mixture of air, water and abrasive particles and thereby breaking down the adherent film of oxide thereon to expose a new surface, the abrasive particles being of from about one hundred mesh to about twelve hundred and fifty mesh, and subjecting said portion of the article to the action of caustic alkali and alkali zincate to produce a deposit of zinc on said portion of the article.

2. The subject matter of claim 1, characterized by the fact said portion of the article is subjected to the alkali and zincate after the completion of the blasting operation.

3. The subject matter of claim 2, characterized by the fact that directly following the blasting operation, and prior to the subjecting of the article to the alkali and zincate, the portion of the article to be electroplated is subjected to at least one solution of at least one strong mineral acid.

4. The subject matter of claim 1, characterized

by the fact that said alkali and zincate operation is performed subsequent to said blasting operation, thereafter the portion of the article to be electroplated is subjected to at least one solution of at least one strong mineral acid, and thereafter said portion of the article is subjected again to the action of caustic alkali and alkali zincate to produce a deposit of zinc on said portion of the article.

5. The method of producing a deposit of metal on aluminum which comprises treating the aluminum in accordance with claim 4, and thereafter electroplating the metal on the portion of the aluminum that has been so treated.

6. The subject matter of claim 1, characterized by the fact that in addition to subjecting the area to be plated to blasting and to alkali and zincate, said portion of the article, subsequent to the blasting, is subjected to the action of at least one solution of at least one strong mineral acid and the last significant step in the preparation for electroplating consists in subjecting said portion of the article to the action of an aqueous solution of caustic alkali and alkali zincate.

7. The method of producing a deposit of metal on aluminum, which comprises treating the aluminum in accordance with claim 1, and thereafter electroplating the metal on that portion of the aluminum that has been so treated.

KUNO L. VAN DER HORST.

#### References Cited in the file of this patent

#### UNITED STATES PATENTS

| Number    | Name       | Date          |
|-----------|------------|---------------|
| 1,627,900 | Hewitson   | Mar. 10, 1927 |
| 1,923,790 | Moore      | Aug. 22, 1933 |
| 1,984,624 | Bagley     | Dec. 18, 1934 |
| 1,988,645 | Bowden     | Jan. 22, 1935 |
| 2,142,564 | Korpium    | Jan. 3, 1939  |
| 2,414,923 | Batcheller | Jan. 28, 1947 |

#### OTHER REFERENCES

The Monthly Review of American Electroplaters' Society, March 1946, pages 269, 270, 273, 274, 277.

Metal Finishing, February 1949, pages 48-53.